

Aug. 10, 1926.

1,595,745

W. TRURAN

COAL CONCENTRATION

Filed May 24, 1922



INVENTOR  
*William Truran*  
BY *William & Prochard*  
ATTORNEYS

Patented Aug. 10, 1926.

## UNITED STATES PATENT OFFICE.

WILLIAM TRURAN, OF YOLANDA, CALIFORNIA, ASSIGNOR TO MINERALS SEPARATION  
NORTH AMERICAN CORPORATION, OF NEW YORK, N. Y., A CORPORATION OF  
MARYLAND.

## COAL CONCENTRATION.

Application filed May 24, 1922. Serial No. 563,341.

This invention relates to the froth-flotation concentration of coal-bearing materials and enables the self-frothing characteristics of many coal-bearing materials to be utilized so as to effect economy in the consumption of agents used in the process.

Since coal is in almost all parts of the world a relatively cheap material, the cost of the reagents used in effecting froth-flotation concentration of the coal becomes an important item where such concentration is necessary or is advisable for any purpose.

According to the present invention, instead of adding a frothing agent to the pulp of ground coal and water at the beginning of the operation, the concentration is commenced by agitating and aerating the coal pulp in the usual manner for froth-flotation concentration, without the addition of an agent, so that a substantial portion of the coal is raised in a coal-bearing froth. An agent is then added to the depleted pulp and the concentration of the coal completed by further agitation and aeration to produce further coal-bearing froth. The coal-bearing froths are separated from the pulps in the usual manner and the entire operation may be continuous. It is found that by working in this manner, the amount of added agent used to effect the complete concentration of the coal is substantially reduced with resulting economy.

The examples herein described were carried out in a subaeration machine of the kind shown in sectional side view in the accompanying drawing.

This machine has an agitation chamber 1, of rectangular cross-section, provided with an agitator 2 turning near the bottom of the chamber and carried by a shaft 3, which is journaled in overhead bearings 4 and 5, and has a driving pulley 6, at the top, and is supported just below the pulley by a suitable thrust bearing 7.

To form a froth, the agitator 2 is driven in the proper direction at a suitable speed and air is thereby drawn in through a bottom pipe 9, suitably connected by a U-extension to an upright pipe 10, extending above the level of the pulley in the chamber 1 and provided with a valve 11 to control the admission of air beneath the agitator 2. A suitable baffle 12 is located above the agitator 2, and is shown as formed of intersecting

metal sheets 13 and 14, set at right angles 55 to each other.

Alongside of the agitation chamber 1 is formed a spitzkasten 18 and the wall 17 between the agitation chamber and the spitzkasten terminates at the top below the pulp level, and provides communication at the bottom between the agitation chamber and spitzkasten, thus permitting the pulp to flow over the top of this partition into the spitzkasten and to flow downward and back 60 from the spitzkasten into the agitation chamber.

A draining opening 24, closed by a plug 25, is located in the bottom of the agitation 70 chamber.

The following are examples of procedures embodying my invention:

1. 500 grams of coal of the Cambria Steel Company, suitably ground to pass a ten-mesh Tyler screen, was made into a pulp 75 with water and agitated and aerated for five minutes without the addition of any agent and a coal-bearing froth formed. There was then added 0.3 pounds per ton of commercial cresylic acid and 0.6 pounds 80 per ton of Eastern fuel oil. Agitation was continued for another five minutes, and further coal-bearing froth was formed. The overflow of froth was continuous from the first formation thereof to the end of the 85 total ten-minute period of agitation. The concentrate thus obtained was further treated by reagitation for ten minutes in the same machine to produce a cleaner froth with addition of 0.1 pound per ton of the same 90 cresylic acid, 0.5 pounds per ton of the same Eastern fuel oil, and 0.4 pounds per ton of starch, the latter being added in the form of a thin paste. The results are shown 95 in the following table:

|               | Wt. % | % Ash. | % S. | Grms. good coal. | % Recovery good coal. | 100 |
|---------------|-------|--------|------|------------------|-----------------------|-----|
| Heads.....    | 100.0 | 11.8   | 2.19 | 355.0            | 99.6                  |     |
| Conc.....     | 88.6  | 6.8    | 0.99 | 353.4            |                       |     |
| Tailings..... | 11.4  | 55.0   | 11.5 | 1.6              |                       |     |

2. 500 grams of coal from the Freeport seam of the American Manganese Manufacturing Co. mine was ground to pass through a ten-mesh standard Tyler screen and was agitated for three minutes in the same ma- 105

chine without the addition of any agent, forming a coal-bearing froth. There was then added 0.4 pounds per ton each of the same cresylic acid and Eastern fuel oil and

5 agitation was continued for three minutes, forming further coal-bearing froth. The total overflowing froth was collected. The results are shown in the following table:—

| 10.           | Wt. % | % Ash. | % S. | Grms. good coal. | % Recovery good coal. |
|---------------|-------|--------|------|------------------|-----------------------|
| Heads-----    | 100.0 | 14.3   | 1.43 | 290              | -----                 |
| Conc.-----    | 86.6  | 7.2    | 1.09 | 288              | 99.3                  |
| Tailings----- | 13.4  | 60.6   | 2.91 | 2                | -----                 |

15

3. 500 grams of coal from the American Manganese Manufacturing Company was ground to pass through a ten-mesh standard

20 Tyler screen, and was agitated for three minutes without the addition of any agent and a coal-bearing froth formed. There was then added 1.3 pounds per ton of Eastern fuel oil. Agitation was continued for another five minutes, and further coal-bearing

25 froth was formed. The overflow of froth was continuous from the first formation thereof to the end of the total ten-minute period of agitation. The results are shown in the following table:—

| 30         | Wt. % | % Ash. | % S. | Grms. good coal. | % Recovery good coal. |
|------------|-------|--------|------|------------------|-----------------------|
| Heads----- | 100.0 | 13.9   | 65.1 | 325.5            | -----                 |
| Conc.----- | 77.9  | 7.4    | 79.0 | 307.9            | 94.3                  |
| Tails----- | 22.1  | 36.6   | 15.9 | 17.6             | -----                 |

35 It is obvious that in the embodiment of this invention in the concentration of coal-bearing materials to which it is applicable, the agents used and the proportions in which they are added and the details of operation will be adjusted to the particular requirements in each instance as determined by test and trial as is well known in this art.

40 I claim:

1. The process of concentrating coal-bearing material which consists in agitating and aerating a pulp of the suitably ground material to produce a coal-bearing froth without addition of an agent, then adding an agent to the depleted pulp and subject-

45 ing the depleted pulp to further agitation and aeration to form further coal-bearing froth, and separating the froths from the 55 pulps.

2. The process of concentrating coal-bearing material which consists in agitating and aerating a pulp of the suitably ground material to produce a coal-bearing froth 60 without addition of an agent, then adding an oily agent to the depleted pulp and subjecting the depleted pulp to further agitation and aeration to form further coal-bearing froth, and separating the froths from 65 the pulps.

3. The process of concentrating coal-bearing material which consists in agitating and aerating a pulp of the suitably ground material to produce a coal-bearing froth 70 without addition of an agent, then adding an oil and a soluble frothing agent to the depleted pulp and subjecting the depleted pulp to further agitation and aeration to form further coal-bearing froth, and separating the froths from the pulps.

4. The process of concentrating coal-bearing material which consists in agitating and aerating a pulp of the suitably ground material to produce a coal-bearing froth 75 without addition of an agent, then adding a petroleum oil and a soluble frothing agent to the depleted pulp and subjecting the depleted pulp to further agitation and aeration to form further coal-bearing froth, and separating the froths from the pulps.

5. The process of concentrating coal-bearing material which consists in agitating and aerating a pulp of the suitably ground material to produce a coal-bearing froth 80 without addition of an agent, separating the froth from the pulp, then adding an oily agent to the depleted pulp and subjecting the depleted pulp to further agitation and aeration to form further coal-bearing froth 85 and separating this froth from the pulp, then reagitating and reaerating the commingled froths with the addition of a small quantity of starch to form a cleaner froth, and separating the cleaner froth.

90 In testimony whereof, I have affixed my signature to this specification.

100 WILLIAM TRURAN.